

Sept. 13, 1960

K. ZIEGLER ET AL  
PURIFICATION OF ALUMINUM

2,952,589

Filed April 4, 1957

3 Sheets-Sheet 1



INVENTOR.  
KARL ZIEGLER, HANS HERBERT LEHMKAUL  
BY  
Burgers, Dinklage & Grunig  
ATTORNEYS

Sept. 13, 1960

K. ZIEGLER ET AL  
PURIFICATION OF ALUMINUM

2,952,589

Filed April 4, 1957

3 Sheets-Sheet 2



INVENTORS.  
KARL ZIEGLER, HANS HERBERT LEHMKUHL  
BY  
*Burgen, Dinklage & Spengler*

ATTORNEYS

Sept. 13, 1960

K. ZIEGLER ET AL

2,952,589

PURIFICATION OF ALUMINUM

Filed April 4, 1957

3 Sheets-Sheet 3



Fig. 5a



Fig. 5b

INVENTOR.  
KARL ZIEGLER, HANS-HERBERT LEHMKUHL  
BY  
*Bürgers, Dunklau & Speng*  
ATTORNEYS

# United States Patent Office

2,952,589

Patented Sept. 13, 1960

1

2,952,589

## PURIFICATION OF ALUMINUM

Karl Ziegler, Kaiser Wilhelm Platz 1, Mulheim (Ruhr), Germany, and Hans-Herbert Lehmkuhl, Mulheim (Ruhr), Germany; said Lehmkuhl assignor to said Ziegler

Filed Apr. 4, 1957, Ser. No. 650,709

Claims priority, application Germany Apr. 9, 1956

16 Claims. (Cl. 204—14)

This invention relates to new and useful improvements in the purification of aluminum.

With the recent developments in the chemistry of organo-aluminum compounds, various proposals have been made for the recovery of extremely pure aluminum from impure aluminum using organic aluminum compounds such as aluminum alkyls as intermediates.

In accordance with one such proposal, pure aluminum is recovered at the cathode of an electrolysis cell having an anode of impure aluminum and an  $\text{NaF} \cdot 2\text{Al}(\text{C}_2\text{H}_5)_3$  electrolyte.

In accordance with another proposal and in contrast to the above-mentioned electrolytic process, pure aluminum is produced in a strictly thermal process. The impure aluminum is dissolved by means of isobutylene and hydrogen forming tri-isobutyl aluminum which is, first of all, thermally decomposed into diisobutylaluminum hydride and iso-butylene and thereafter further decomposed into the pure aluminum, hydrogen and isobutylene.

The above described electrolytic process involves certain difficulties since a current density of more than about 1 ampere per square decimeter cannot be exceeded without mechanically treating the cathode surface during the electrolysis. In addition, the electrolyte has a relatively low conductivity (about  $4 \cdot 10^{-2} \text{ ohm}^{-1} \text{ cm.}^{-1}$  at  $140^\circ \text{ C.}$ ) so that the cathodes and anodes must be maintained relatively close to each other in the cell in order to obtain the advantage of a small energy consumption. This close proximity of the cathodes and anodes, however, results in difficulties with respect to maintaining contaminates from the anode away from the cathode.

In the above described thermal process, difficulties are encountered since large quantities of gas must be handled. For each gram of aluminum formed, 33 normal liters of gas are produced which must be circulated. In addition, difficulties are encountered in removing the aluminum in a well adhering compact form.

One object of this invention is a combination, non-electrolytic-electrolytic process for the purification of aluminum without the above-mentioned difficulties. This, and still further objects, will become apparent from the following description read in conjunction with the drawings in which:

Figure 1a is a diagrammatic plan view of an apparatus for effecting the process in accordance with the invention,

Figure 1b is a diagrammatic vertical section of an apparatus for effecting the process in accordance with the invention,

Figure 2 is a diagrammatic plan view of a series of electrolysis cells for effecting the process in accordance with the invention,

Figure 3 is a diagrammatic side elevation of a still further embodiment of an apparatus for effecting the process in accordance with the invention,

Figure 4 is a diagrammatic vertical section of a still further embodiment of an apparatus for effecting the process in accordance with the invention with the formation of large compact pieces of purified aluminum,

2

Figure 5a is a diagrammatic side elevation of a still further embodiment of an apparatus for effecting the process in accordance with the invention with the formation of compact purified aluminum bars, and

5 Figure 5b is a diagrammatic plan view of the apparatus shown in Figure 5a.

In accordance with the invention, the purification of the aluminum is effected by contacting the impure aluminum in a first stage with a lower aluminum trialkyl and hydrogen to thereby form a lower dialkyl aluminum hydride. The lower dialkyl aluminum hydride thus formed in the first stage is mixed with an electrically conductive complex organic aluminum compound forming an electrolyte and the electrolyte mixture or solution thus formed is electrolyzed in a second stage in an anode-cathode containing electrolysis cell forming pure aluminum at the cathode and hydrogen at the anode.

In the first stage the conversion of the aluminum into the soluble organic aluminum compound proceeds in 20 accordance with the equation



in which R represents a lower alkyl radical. As the 25 aluminum is not directly converted into a trialkyl aluminum, a special unsaturated hydrocarbon is not required and, in addition to the starting aluminum trialkyl, only hydrogen is required.

While any lower aluminum trialkyl, as for example 30 ranging from trimethyl aluminum to tributyl or isobutyl aluminum, may be used as the starting aluminum trialkyl, it has been found preferable to use triethyl aluminum since, due to its low molecular weight, it permits the best utilization of the reaction spaces under pressure and is readily obtainable. Trimethyl aluminum, while theoretically being more favorable due to its even lower molecular weight, is not at present as readily available as the triethyl aluminum. As mentioned, other lower aluminum alkyls, as for example, tripropyl, tri-isobutyl 40 or tri-butyl aluminum may also be used.

The dialkyl aluminum hydrides, such as the diethyl 45 aluminum hydride, thus formed is not a conductor of electricity and therefore cannot be used as such in the electrolysis of the second stage. In accordance with the invention, however, it has been found that by mixing the lower dialkyl aluminum hydrides such as the diethyl aluminum hydride with electrically conductive complex aluminum compounds, and preferably alkali metal organic aluminum compound such as sodium halide, lower aluminum trialkyl complexes, as for example



lower alkali metal aluminum tetra alkyl complexes as, for example, sodium aluminum tetraethyl or alkali halide lower dialkyl aluminum halide complexes, as for example 55  $\text{KCl} \cdot \text{Al}(\text{C}_2\text{H}_5)_2\text{Cl}$ .

The electrically conductive complex organic aluminum compounds must, of course, be miscible with the dialkyl aluminum hydride forming an electrically conductive mixture or solution having a conductivity, for example, 60 of the order of magnitude of  $1 \cdot 4 \cdot 10^{-2} \text{ ohm}^{-1} \text{ cm.}^{-1}$ . The conductivity of these mixtures or solutions can, furthermore, be favorably affected by increasing the temperature at which the electrolysis is effected.

Upon the electrolysis in a cathode-anode containing 65 electrolysis cell, very pure aluminum is deposited at the cathode and hydrogen form at the anode. The hydrogen should be liberated, i.e., bubble off the anode so that the anode metal should be one which does not react with hydrogen as, for example, iron, stainless steel or preferably copper or silver. If aluminum anodes are used, the hydrogen will not be liberated but rather a corresponding

quantity of aluminum will pass into solution. Aluminum anodes therefor cannot be used in accordance with the invention.

As long as a certain minimum content of the dialkyl aluminum hydride is maintained in the electrolyte, the complex aluminum compounds which render the electrolyte conductive, are not changed during the course of the electrolysis. The electrolysis is therefore simply a reversal of the formation of the dialkyl aluminum hydride and for each three mols of the dialkyl aluminum hydride, 2 mols of the trialkyl aluminum, 1.5 mols of hydrogen and 1 gram atom of pure aluminum are formed.

Since the dialkyl aluminum hydride is initially produced from aluminum, hydrogen and trialkyl aluminum, the same may be considered as being produced from aluminum hydride and trialkyl aluminum and the electrolysis can be considered as nothing more than the breaking down of this aluminum hydride into aluminum and hydrogen.

The trialkyl aluminum, such as triethyl aluminum, liberated during the electrolysis, is not miscible to the same extent with the complex aluminum compounds which conduct the current as the dialkyl aluminum hydride is. Accordingly, the trialkyl aluminum separates during the electrolysis in the form of an insoluble upper layer which may still contain small quantities of the dialkyl aluminum hydride. This separated upper layer may very easily be removed from the electrolysis and recycled to the first reaction stage for the reaction with the crude aluminum and hydrogen to form the dialkyl aluminum hydride for the electrolysis.

When considering the process in accordance with the invention as a whole, therefore, the trialkyl aluminum is not consumed and is merely recycled between the stages acting, in effect, as a dissolving intermediate for the aluminum by the hydrogen. Additionally the hydrogen used in the first stage is not lost but is reformed again during the electrolysis at the anode and may be recovered, compressed and reused again in the first reaction stage. The only material that need be supplied to the reaction is, therefore, the crude aluminum which is converted into the purified aluminum. It is thus apparent that the entire process may be considered as a simple formation of aluminum hydride, stabilized by reaction with the trialkyl aluminum, and the re-decomposition of the aluminum hydride into a purified aluminum and hydrogen with the recycling of the hydrogen and the trialkyl aluminum to the first stage for the formation of further quantities of aluminum hydride.

The electrolysis, in accordance with the invention, using the lower dialkyl aluminum hydride—electrically conductive organic aluminum complex electrolyte—is highly advantageous. The inert metallic anodes may be positioned in the electrolysis cell very close to the cathodes without fear of contamination and the elemental hydrogen which is liberated will in no way disturb the cathode process. As a result of this, high current densities of up to 20 amps. per square decimeter, as for example 5 to 20 amps. per square decimeter, may be obtained with low cell voltages of, for example, 0.5 to 1 volt so that the energy consumption in the electrolysis is almost insignificant. With the use of such high current densities, the cells may very easily be constructed so that, with the use of certain additional mechanical measures, the aluminum may be recovered in a compact form. Additionally the anodes and cathodes may be ideally shaped with respect to each other and their function whereas in the purely electrolytic refining with the use of anodes of crude aluminum this is impossible due to the difficulties encountered in keeping contaminates from the anode away from the cathode.

The purified aluminum may be recovered in various forms depending upon the mode of operation in accordance with the invention. Thus, for example, the refined aluminum may be recovered in the form of a finely or

coarsely crystalline powder or else in compact form as desired.

In normal operation the purified aluminum may be removed from the cathode in a finely crystalline form which becomes more coarsely crystalline as a function of the time during which the same remains in the electrolyte. A purified aluminum powder of the desired crystal size may, therefore, be obtained merely by a suitable selection of the time interval at which the powder is removed from the electrolyte.

It is also possible to recover the aluminum in a compact form by mechanically pressing the same on the cathode during the electrolysis.

Referring to the embodiment of the electrolysis cell as shown in Figures 1a and 1b of the drawings, the cathodes of this cell are in the form of a series of vertically positioned parallel metallic rollers C which are spaced apart and which do not contact each other. These rollers are mounted for rotation on suitable bearings, not shown, and are rotated, preferably at a uniform rate of speed, by suitable drive means as, for example, an electric motor (not shown). Anodes B of, for example, iron, stainless steel, copper, some other suitable metal, are positioned closely adjacent to the cathodes and have convex curved portions corresponding in shape to the cylindrical shape of the cathodes. On the opposite side of the anodes, scrapers A are positioned in contact with the surface of the roller shaped cathodes C so that, as the cathodes rotate, the scrapers A will scrape off the pure aluminum which deposits during the electrolysis.

The cathodes, anodes and scrapers are positioned in the container X which is filled with the lower dialkyl aluminum hydride—electrically conductive complex organic aluminum compounds electrolyte—so that the liquid electrolyte surrounds the cathode and is in contact with both the cathode and anode in the conventional manner.

A bell shaped gas collector D provided with an exhaust conduit leading, for example, to a compressor, may be positioned above the anodes in order to collect the hydrogen evolved during the electrolysis. The hydrogen so withdrawn and compressed may be recycled to the first stage for the formation of the dialkyl aluminum hydride. It is also possible to fill the space above the cathodes with a suitable protective gas as, for example, nitrogen.

In operation, a direct current is applied across the cathode and anode as the cathodes are rotated in contact with the scrapers A. The pure aluminum which deposits on the cathodes as a result of the electrolysis is removed by the scrapers A and deposited at the bottom of the container X which preferably has a trough-shaped channel for receiving this loose crystalline aluminum. The fineness of the original deposit of aluminum is maintained under the liquid electrolyte in the cell, its coarseness increases as a function of time so that the degree of division of the recovered aluminum can be controlled by a suitable selection of the period of time during which the same is maintained in the electrolyte prior to removal.

The aluminum trialkyl which forms as an upper layer during the electrolysis may be continuously or intermittently removed and recycled to the first stage for the formation of dialkyl aluminum hydride and replaced by a corresponding quantity of the dialkyl aluminum hydride insuring continuous operation.

For reasons of economy it is desirable to use the highest current densities possible. The electrolysis cell is, for example, operated at current densities of between 5 and 20 amps. per square decimeter and the anode may be positioned within a few millimeters of the rotating cathode. With a specific conductivity of the electrolyte of  $3 \cdot 10^{-2} \text{ ohm}^{-1} \text{ cm.}^{-1}$ , a current of 10 amps. may be maintained per square decimeter of electrode surface at a voltage of 1 volt. The speed of rotation of the cathode

rollers should, of course, be so adjusted that the growing layer of the loosely adherent aluminum does not reach the anode during one revolution and thus is continuously scraped off before the same will short the anode and cathode.

It is preferable to effect the electrolysis using a long row of the cells as shown in Figures 1a and 1b positioned one after the other in a closed space which is filled with hydrogen upon the placing of the cells in operation and in which the hydrogen formed upon the electrolysis collects and may be removed. The hydrogen which collects in this space may be withdrawn by means of a compressor and recycled to the first stage for the production of the dialkyl aluminum hydride.

The troughs at the bottom of the containers X to which the scraped off aluminum collects, may be positioned adjacent to one another forming a common elongated trough from which the aluminum may be continuously or intermittently removed by means of a suitable device as, for example, a conveyor, a scraper flights, a grab bucket, or the like.

As shown in Figure 2, a multiple number of the cells are positioned alongside one another in a long row and provided with a grab bucket G which moves on the crane runway E through the elongated trough formed by the individual troughs of the containers X and removes the loose aluminum which has been scraped off from the cathodes. The time of movement of the grab bucket G may be controlled to obtain the desired crystalline size of the aluminum and the removed aluminum is deposited in the discharge device F as, for example, in the form of a lock chamber which allows the removal of the aluminum without contact with the air. If desired, traces of the electrolyte which still adhere may be washed out from the aluminum by means of a hydrocarbon solvent as, for example, benzene, and the aluminum may be pressed into the form of compact pieces as, for example, in cylindrical molds and thereafter melted down in a suitable manner.

The individual cells may be flow connected so that a common removal of the formed trialkyl aluminum and a common introduction of a corresponding amount of the dialkyl aluminum hydride may be effected.

Instead of cathodes in the form of rotating cylinders or rollers, other moving cathode shapes may, of course, be used. Thus, for example, as shown in Figure 3, the cathode may be in the form of an endless metal belt H which is stretched over to rollers I, at least one of which is driven by suitable drive means as, for example, an electric motor. The anode B is in the form of a suitable screen or grid which extends over the horizontally moving portions of the endless cathode belt H. The deposited aluminum may be removed by the scrapers A and if the scraper A is provided at each reversal point, i.e., at each of the rollers, both sides of the cathode belt H may be utilized for the depositing of the aluminum. The entire arrangement is positioned in a suitable vessel as, for example, one corresponding to the vessel or container X of Figure 1b, immersed in an electrolyte and a direct current potential is applied between the cathode belt H and the anode D.

If it is desired to deposit the purified aluminum on the cathode in a compact form, it is merely necessary to press the same in contact with the cathode surface during the electrolysis as, for example, by means of rollers or the like. This is even desirable at low current densities as, for example, of the order of magnitude of 1 amp. per square decimeter since even at these low current densities the aluminum layer on the cathode, without mechanical compression, will grow, becoming coarsely crystalline and finally becoming covered with pimply irregularities. As mentioned, for reasons of economy, it is desirable to operate at as high a current density as is possible and at these higher current densities, the necessity of mechanical pressure in order to obtain a thick layer

of aluminum on the cathode is even more pronounced.

The mechanical pressing is most simply done by rolling the cathode with a roller of an insulating material as, for example, glass, porcelain, sintered aluminum, hard wood, Teflon or the like. Thus, for example, in Figures 1a and 1b the scrapers A may be replaced by pressure rollers of a suitable insulating material. It is also preferable to provide an arrangement so that the anode and cathodes may move away from each other as the aluminum coating on the cathode rollers increases, thus preventing shorting.

Due to the convex shaping of the anode, there is a limitation as to the thickness of the aluminum coating which can be built up in this manner. After the aluminum coating has grown to the desired or maximum size, the same must be removed as, for example, by the removing of the cathodes themselves and replacing with fresh cathodes. If the starting cathodes are themselves pure aluminum, a separation of the deposited aluminum from the cathode is not necessary.

20 An embodiment of an apparatus, in accordance with the invention, which is particularly well suited for the production of large compact pieces of refined aluminum, is shown in Figure 4. The cell as shown in the form of elongated, horizontally extending vessel or container

25 X which is provided with a hydrogen outlet at its upper portion leading, for example, to a compressor not shown. The lower portion of the container X is filled with the electrolyte and provided with the flat cathode plate L at the central portion of its bottom.

30 The anode is in the form of a flat grid or screen which is supported by means of a frame or chassis mounted on the rollers K of a suitable insulating material.

During operation, the rollers K are rolled back and forth over the cathode L by means of a suitable reciprocating drive, not shown. The direct current is applied across the cathode L and the anode M. The anode M is of a suitable size so that the same will completely cover the cathode L at each limit of back and forth movement of the rollers K and the chassis mounted thereon.

35 40 In addition, dead spaces with the platforms N are provided on which the rollers K can roll in each direction of movement. The bases N are so provided that the same may be raised to provide a flat rolling surface for the rollers K as the height of the cathode L grows due to the depositing of the aluminum.

45 The layer of the dialkyl aluminum hydride containing electrolyte need, for example, only be a few centimeters above the cathode L. Since distance of the anode M from the cathode L is at all times constant during operation, the layer of aluminum which forms and is compacted on the cathode L may grow to a considerable thickness over a prolonged period of operation.

50 The dialkyl aluminum hydride containing electrolyte is preferably introduced at one side of the cell and removed at the other and the trialkyl aluminum produced is allowed to separate in a special device for this purpose as, for example, a separating vessel, centrifuge, or the like. The electrolyte is then regenerated by the further addition of dialkyl aluminum hydride and recycled to the

55 60 cell while the recovered trialkyl aluminum is recycled to the first reaction stage for the formation of further quantities of dialkyl aluminum hydride.

A plurality of cells, as shown in Figure 4, may be arranged in series one behind the other and it is possible, without difficulty, to produce blocks of the purest aluminum of several square meters surface and a thickness of, for example, 6 centimeters upon continuous operation as, for example, for ten days with a consumption of energy of only about 1 kilowatt hour per kilogram. It is extremely easy, after the long period of operation, to drain the electrolyte from the cell, wash the cell with an inert solvent as, for example, a hydrocarbon, and to remove the aluminum block. The flat cathode L is advisedly a metal to which the aluminum adheres poorly as, for ex-

ample, steel, steel alloys or the like. The flat bottom of the cell itself may be the cathode or a removable metal plate may be placed at the bottom of the cell and lifted out with the aluminum block and later separated therefrom. If a cathode plate is used which is, of itself, pure aluminum, a separation is, of course, not necessary.

In the embodiment, as shown in Figures 5a and 5b, an endless rotating belt P is provided which rotates around two parallel, spaced-apart rollers driven by suitable drive means not shown. A number of parallel, spaced-apart metal strips which preferably consist of very pure aluminum are positioned transversely across the belt P and serve as the cathodes. Anodes in the form of grids or screens B are positioned parallel to and slightly spaced from the horizontally extending portions of the belt P. The belt P and strips O pass between two pairs of compression rollers K of suitable insulating material.

In operation, the entire arrangement is immersed in an electrolyte solution in a vessel as, for example, of the type shown in Figure 4 and a direct current potential is applied between the anode B and the cathode strips O. The endless belt is rotated by driving one or both of the spaced-apart rollers and, as the strips pass the anode B, aluminum deposits thereon and is compressed into a compact form by compression rollers K. After the aluminum layer is built up in compacted form to a suitable thickness on the strips O the same may be removed at R during operation and fresh strips inserted at Q. If desired, a device may be provided which will automatically remove the strips of a given thickness at R and replace the same with new cathode plates at Q. If the initial cathode strips consist of the same very pure aluminum as is obtained by the electrolytic depositing, the same, upon removal, may be immediately melted for use or melted after the removal of any residual electrolyte as, for example, by washing with a hydrocarbon solvent such as benzene. In place of plates, sheets of very pure aluminum may, of course, be produced in the same manner.

The pure aluminum produced in accordance with the invention is of excellent quality and characterized by an extremely high resistance to corrosion.

The following examples are given by way of illustration and not limitation:

#### Example 1

Impure aluminum, hydrogen and triethyl aluminum are contacted in a molar ratio of 1:1.5:2 forming diethyl aluminum hydride. 258 grams (3 gram mols) of the diethyl aluminum hydride thus formed is combined with 270 grams (1 gram mol) of  $\text{NaF}\cdot2\text{Al}(\text{C}_2\text{H}_5)_3$ , forming an electrolyte of the composition



The electrolyte thus prepared is filled into an electrolysis cell corresponding to that shown in Figure 1b provided with a silver anode and maintained at about 80° C. A direct current is supplied across the anode and cathode forming a current density of 0.5 to 10 amps. per square decimeter. Pure hydrogen is given off at the anode and a finely crystalline pure aluminum accumulates at the cathode which is scraped off. The aluminum is continuously scraped from the cathode, removed from the cell, washed with benzene to remove any traces of the electrolyte and thereafter pressed and melted and formed into bars which are extremely pure and corrosion resistant. The hydrogen may be recovered from the anode by compression and recycled for the contacting with the aluminum triethyl. Additionally, during operation of the cell an upper layer of aluminum triethyl forms which may be removed and recycled for contacting with the hydrogen and crude aluminum for the formation of the diethyl aluminum hydride. A corresponding quantity of the diethyl aluminum hydride may be added to the cell to replace a quantity of the aluminum triethyl removed.

#### Example 2

One gram mol (270 grams)  $\text{NaF}\cdot2\text{Al}(\text{C}_2\text{H}_5)_3$  and 0.5 gram mol (43 grams) of  $\text{HAl}(\text{C}_2\text{H}_5)_2$  are mixed, forming an electrolyte with the composition  $\text{NaF}\cdot2\text{Al}(\text{C}_2\text{H}_5)_3\cdot0.5\text{HAl}(\text{C}_2\text{H}_5)_2$ . The diethyl aluminum hydride is formed by contacting hydrogen, triethyl aluminum and crude aluminum.

Electrolysis is effected with this electrolyte at a temperature of about 120° C. in an electrolysis cell having a copper anode and operated at a current density of 10 amps. per square decimeter. Practically pure hydrogen, contaminated only with about 1.0 to 0.5% of a mixture of ethane and ethylene, is generated at the anode and very pure aluminum is deposited at the cathode. The quantity of hydrogen formed at the anode is equal to that which may be calculated from the quantity of the current used.

#### Example 3

Example 2 is repeated except that the electrolysis is effected with the electrolyte at a temperature of about 150° C. Pure hydrogen is obtained at the anode and very pure aluminum is deposited at the cathode. The aluminum may be scraped off the cathode as a finely crystalline powder, the coarseness of which increases as the same is maintained under the electrolyte for a period of time.

#### Example 4

One gram mol (354 grams)  $\text{NaF}\cdot2\text{Al}(\text{C}_3\text{H}_7)_3$  and 2 gram mols (228 grams) of  $\text{HAl}(\text{C}_3\text{H}_7)_2$  are mixed, forming an electrolyte of the composition



The tripropyl aluminum hydride is initially formed by contacting impure aluminum, hydrogen and tripropyl aluminum. Electrolysis is effected with this electrolyte at a temperature of 100° C. in an electrolysis cell using a silver anode and a current density of 5 amps. per square decimeter. Pure hydrogen is generated at the anode and very pure aluminum deposits at the cathode. During the depositing, the aluminum is continuously compressed by rolling the same with a glass roller. A very compact pure aluminum mass is thus formed at the cathode.

While the invention has been described in detail with reference to the specific embodiments, various changes and modifications which fall within the spirit of the invention and the scope of the appended claims will become apparent to the skilled artisan.

We claim:

1. Process for the purification of aluminum which comprises contacting the aluminum to be purified with a lower aluminum trialkyl and hydrogen to thereby form a lower dialkyl aluminum hydride, mixing said lower dialkyl aluminum hydride with an electrically conductive complex organic aluminum compound miscible therewith to thereby form an electrolyte, passing an electric current through said electrolyte between a cathode and an anode selected from the group consisting of silver and copper in an electrolysis cell to thereby electrolyze the electrolyte forming pure aluminum at the cathode, hydrogen at the anode, and an upper layer of aluminum trialkyl, and recycling said aluminum trialkyl and said hydrogen formed at the anode for said contacting with the aluminum to be purified to form said lower dialkyl aluminum hydride.

2. Process according to claim 1 in which said complex organic aluminum compound is an alkali metal organic aluminum complex.

3. Process according to claim 1 in which said complex organic aluminum compound is a member selected from the group consisting of sodium halide-lower aluminum trialkyl complexes, alkali metal-lower aluminum tetraalkyl complexes and alkali metal halide-lower dialkyl aluminum complexes.

4. Process according to claim 1 in which said complex organic aluminum compound is  $\text{NaF} \cdot 2\text{Al}(\text{C}_2\text{H}_5)_3$ .  
 5. Process according to claim 1 in which said complex aluminum compound is sodium aluminum tetraethyl.

6. Process according to claim 1 in which said aluminum trialkyl is triethyl aluminum.

7. Process according to claim 1 in which said electrolysis is effected with a current density of between about 5 to 20 amps. per square decimeter and a cell voltage between about 0.5 and 1 volt.

8. Process according to claim 7 in which said electrolysis is effected with the anode positioned closely adjacent the cathode in the electrolysis cell.

9. Process according to claim 1 which includes scraping the pure aluminum formed from the cathode during said electrolysis.

10. Process according to claim 1 which includes maintaining the aluminum formed at the cathode in the electrolyte for a period of time sufficient to increase the size of its crystal structure and thereafter removing the same from the electrolyte.

11. Process according to claim 1 which includes maintaining a protective inert gas above the cathode during said electrolysis.

12. Process according to claim 1 which includes compressing the aluminum formed on the cathode into a compact structure during said electrolysis and thereafter recovering the compacted aluminum.

13. Process according to claim 12 which includes washing the recovered aluminum with a hydrocarbon solvent and thereafter melting the same.

14. Process according to claim 11 which includes recovering said pure aluminum from the cathode, washing the recovered aluminum with a hydrocarbon solvent and thereafter melting the same.

15. Process according to claim 1 in which the alumi-

num to be purified is substantially continuously reacted with said lower aluminum trialkyl and hydrogen, the hydride formed substantially continuously passed in admixture with an electrically conductive complex organic aluminum compound, the electrolyte thereby formed substantially continuously passed in and out of electrolysis contact with anode and cathode in the electrolysis cell to thereby substantially continuously deposit purified aluminum at the cathode and in which the hydrogen formed at the anode and the aluminum trialkyl formed are substantially continuously recycled for said contacting with the aluminum to be purified to form the lower dialkyl aluminum hydride, the flow of the reactants and the recycling of the hydrogen and the trialkyl aluminum being so adjusted that the recycled materials are essentially sufficient for the first mentioned reaction with continuously newly added aluminum to be purified.

16. Process according to claim 1, in which said complex organic aluminum compound is  $\text{KCl} \cdot \text{Al}(\text{C}_2\text{H}_5)_2\text{Cl}$ .

20

References Cited in the file of this patent

UNITED STATES PATENTS

|           |                |               |
|-----------|----------------|---------------|
| 1,538,390 | Ewan           | May 19, 1925  |
| 1,911,122 | Keyes et al.   | May 23, 1933  |
| 1,939,397 | Keyes et al.   | Dec. 12, 1933 |
| 2,651,608 | Brenner et al. | Sept. 8, 1953 |
| 2,787,626 | Redman         | Apr. 2, 1957  |
| 2,849,349 | Ziegler et al. | Aug. 26, 1958 |

OTHER REFERENCES

Studies in the Electrodeposition of Metals, Bulletin No. 206, published by University of Illinois, pages 10 and 11.

Angewandte Chemie, vol. 67 (1955), No. 16, pp. 424-426.

35 Chemical Reviews, vol. 54 (October 1954), pp. 844-845.

30